

## UNITED STATES PATENT OFFICE

JACOB LUKASCZYK, OF ROSENBERG, OBERPFALZ, GERMANY

## PROCESS FOR IMPROVING THE HEADS OF RAILWAY RAILS

No Drawing. Application filed August 25, 1927, Serial No. 215,514, and in Germany October 21, 1926.

Attempts to increase the efficiency and economy of railway operation has led to continually higher speeds and continually greater wheel pressures of the locomotives and vehicles. The development of the tracks has however not kept pace with this, and the result thereof is greater wear of the rails, so that more particularly on tracks having sharp curves and steep grades they have only a relatively short length of life. The heavy wear of the rails can be met by thickening the rail profile, or more particularly by employing a steel rail having a higher resistance to wear.

Attempts hitherto made to provide a harder steel rail having a tensile strength of 80 and more kilogrammes per square millimetre have not been satisfactory, because it has been ascertained that resistance to wear and tensile strength are essentially different things. The employment of hard steel, however, such as corresponds to this strength, brings dangers into railway operation, because the hard steel rail no longer has sufficient tenacity, and the prescribed deflection in the bending test is very barely obtained, if at all.

Now it has been found that the resistance of the rails to wear can be enhanced to an extent corresponding to present-day requirements if the steel rail, in the outer zone of the rail head, which is subjected to the greatest wear when being run over, is converted into a texture resembling martensite. This texture shows an unusually great power of resistance to the stresses arising in operation during the practical utilization of the rail, so that rails in which the outer zone of the head is converted into martensite, according to the results of the tests for wear that have been systematically carried out, must have a much longer life than the known rails. It is important, and on the lines of the present invention is attainable, when only the outer zone of the rail head is converted into

martensite, while the rail foot and web are not converted at all, and thereby maintain their high tenacity, which is of the utmost importance in practical operation.

The conversion of the external zone of the rail head into martensite is effected by energetically quenching the warm pieces of rail cut to length, by plunging the rail head into cold water, employing a suitable appliance which prevents warping. This immersion must be of such duration that the rail head assumes a black appearance, and that after being taken out of the bath it does not become red again. After the removal from the bath an improvement of the rail head occurs owing to the heat remaining in the rail foot and the rail web, which have not been cooled.

It has been found that the temperature of the rail head after the quenching should not rise above 450° C., in order that a good result may be ensured.

The appropriate duration for the immersion depends upon the composition of the steel. When working for example with steels having a carbon content of from 0.40 to 0.45 per cent. the time of immersion varies between 1 1/4 and 3/4 minutes, the lower immersion time corresponding to the higher carbon content.

Experiments have shown that the resistance to wear on my treads of rails improved in the rail head by the new process is far more than ten times as great as that of ordinary rails made from the same unimproved material.

What I claim is:—

The process of increasing the resistance of railway rails to wear, said rails having a carbon content between 0.40 and 0.45 per cent, usual in commercial rails, which process comprises, first cutting the rail to the desired length and then plunging the head of the rail while still retaining its rolling heat into cold water for a length of time varying from 1 1/4 minutes for the low carbon content

50

55

60

65

70

75

80

85

90

to  $\frac{3}{4}$  minute for the high carbon content so that the rail-head assumes a black appearance and that the temperature of the rail-head after removal from the water does not exceed 450° C. and does not again become red while the foot and web of the rail remain warm, whereby only the outer zone of the rail-head is given a martensite structure.

5 In testimony whereof I have signed my  
10 name to this specification.

**JACOB LUKASZYK.**

15

20

25

30

35

40

45

50

55

60

65